

W. PETRIE,  
PROCESS OF TANNING.  
APPLICATION FILED APR. 2, 1917.

1,273,662.

Patented July 23, 1918.



Inventor  
Walter Petrie.

Witness  
James F. FitzGibbon.

By K.P. McElroy.  
Attorney

# UNITED STATES PATENT OFFICE.

WALTER PETRIE, OF ENDICOTT, NEW YORK, ASSIGNOR TO PETRIE PROCESS COMPANY,  
OF NEW YORK, N. Y., A CORPORATION OF NEW YORK.

## PROCESS OF TANNING.

1,273,662.

Specification of Letters Patent. Patented July 23, 1918.

Application filed April 2, 1917. Serial No. 159,226.

*To all whom it may concern.:*

Be it known that I, WALTER PETRIE, a subject of the King of Great Britain and Ireland, residing at Endicott, in the county of 5 Broome and State of New York, have invented certain new and useful Improvements in Processes of Tanning, of which the following is a specification.

This invention relates to processes of tanning; and it comprises a method of producing a quick tanning operation wherein hide, which is advantageously first "set", that is treated with tanning solution enough to prevent pebbling or graining in the subsequent 10 operation, is worked with a small quantity of a strong tanning solution, such strong tanning solution being progressively added thereto in small successive portions and the working being advantageously in a drum or 15 the like, the amount of such tanning solution supplied being that which suffices for complete tanning and the strength being such that no substantial excess of liquor or solution remains after the operation, the 20 whole operation being conducted under such conditions as will give sufficient ventilation for cooling and evaporating purposes; all as more fully hereinafter set forth and as claimed.

30 In tanning hides to make leather, all sorts of materials are employed to make the tanning liquors, a tanning action being by no means restricted to what are chemically known as the tannins. These tanning solutions contain materials which have a marked affinity for the hide substance and which may be here called "tans" and bodies which have not this marked affinity and may be called "non-tans". The latter substances 35 however are useful in the leather. In the customary methods of tanning, the hides are treated with a large volume of the tanning liquor, whatever it may be; the bath being replenished with new "extract" from time to 40 time. From this large volume the hides selectively absorb the tans in preference to the non-tans and the non-tans consequently accumulate as the liquor grows older. In the course of time the character of the liquor 45 therefore is apt to change materially. In the tanning, for the sake of quickening the action, agitation of one kind or another is very common. Very frequently the hides are placed in a rotating drum containing a 50 large body of liquor. The agitation due to

rotation materially accelerates the absorption. In view of the large volume of liquor usually employed it is not customary to have it very concentrated; it is, relatively speaking, usually rather dilute. Tanning processes now customary are generally relatively slow. It is the object of the present invention to provide a quicker tanning operation with greater economy of material and a more complete utilization of the tan- 60 65 liquor.

I have found that I can secure a good tanning in a quick way by treating the hides in a rotating drum in the presence of only a small amount of concentrated liquor; merely 70 the amount which suffices to keep the hide more or less wet, adding new concentrated liquor as the hides require it. In so doing I use a type of drum somewhat different from those heretofore employed for tanning purposes, providing means for free ventilation. The ventilation may be that due to natural circulation of air through openings in the drum or it may be a forced ventilation made by passing air through by means of a fan or 75 the like. This free ventilation keeps the material from heating up or becoming warm and also has a useful effect in removing water as vapor, keeping the liquor concentrated. Ordinarily I use merely the amount 80 of strong liquor which will suffice for a complete tanning; using the liquor of such strength that after my operation is completed there is substantially no excess. If there should chance to be a little excess it 85 does no harm since it can be reused; but ordinarily I use just about the amount of liquor which will be absorbed by the hides, allowing for loss due to evaporation. In this method of operation, since I am causing 90 the hide to absorb substantially all the liquor, the liquor I employ must be sufficiently concentrated to afford all the tans and non-tans which it is desired to have taken up by the hide. By the use of strong tan liquors 95 100 I much accelerate the absorption, while the cooling given by the free ventilation and incident evaporation prevents development of heat and injury to the hides. The evaporation also operates to concentrate the liquor 105 further and insure complete absorption. Since the present method puts substantially all the solubles of the "extract" into the hide, preventing the stated differential absorption of tans at the expense of non-tans, I also se-

cure a better utilization of my extract, a greater weight of leather and a uniform product, my product not varying from week to week as is the case in tanning with 5 baths of changing composition.

In the present invention the hides are ordinarily first "set" in a tanning solution, the object of this preliminary treatment not being to tan the hides to any extent but 10 merely to set them enough to prevent graining, etc., in the tanning operation proper; *i. e.*, prevent the surface from becoming puckery or coarse grained. I may take the hides from the beam house and tan them.

15 The hides coming from the setting process which are wet and contain dilute tanning solution are put into a drum together with a little strong tanning solution, say for a 7-foot drum containing 1,500 pounds (wet

20 weight, or what is known as "white weight" among tanners) I add first about 15 to 25 gallons, say 20 gallons of a strong tanning solution, say 220° barkometer or about 30° Bé. The drum is provided with

25 means causing or allowing free ventilation. The drum is rotated and the liquor is taken up by the hides. Evaporation takes place, strengthening the liquor, this evaporation being aided by the free ventilation. As the

30 liquor is absorbed, new strong liquor is added, the time when additions are necessary being judged by the appearance of the leather and liquor. Ordinarily, additions of liquor in small portions are continued at

35 intervals of about 18 to 24 hours, this depending upon the thickness, etc., of the hides; a final period of about 6 to 10 hours rotation being given during which no additions are made. This results in a completely

40 tanned leather with substantially complete absorption of the liquor or extract used. The complete drumming operation takes from about 24 to 36 hours. At no time is there more than enough liquor in the drum than

45 will suffice to keep the leather wet and furnish a little free liquid. The hides are not submerged; neither is a great excess of liquor ever present. Under the conditions, in order to prevent heating there

50 must be, as stated, free ventilation or other methods of cooling.

In the described operation it is better that the materials be somewhat acid; but the amount of acid needed is not great. I 55 do not ordinarily acidify during the tanning operation proper but rely on the presence of enough acid in the hide from the preliminary operation hereinafter described. The acidity may be that due to any mineral 60 or organic acid.

While a wide variety of tanning materials may be employed in the described process, I find that I can operate it very advantageously with various tanning materials comprising or consisting of prepara-

tions from waste sulfite liquor; and particularly that known in the trade as "spruce extract". Spruce extract is a somewhat acidified concentrated waste sulfite liquor. Instead of, or in addition to, spruce extract, however, I may use quebracho, oak, cutch, hemlock, chestnut extracts, etc., or any other well known tanning material. Blends of the various tanning extracts may also be employed.

In an advantageous embodiment of the present invention I take the wet hides coming from the beam house and first color them. This may be done by any of the usual methods.

A good way of doing it 80 is to treat the hides with spruce extract with which may or may not be mingled other tanning materials. Ordinarily I next treat with an acid bath. Any of the ordinary organic or inorganic acids may be em-

ployed. A bath of water containing about 0.2 per cent. sulfuric acid will serve. In this bath the hides may be hung for 24 hours or thereabouts. The hides are next treated in a setting bath which advanta-

geously contains more or less spruce extract. An advantageous strength or solution in the setting operation, using spruce extract, is about 65 barkometer, or, around 9° Bé. It

is advantageous to leave the hides in the 95 setting bath for at least two or three days. If desired, the setting bath and the acid bath may be combined, the setting bath being simply acidified with any convenient acid.

From the setting bath the material 100 next goes to a rotary drum provided with ventilating means of some type wherein it is treated with successive small additions of concentrated tanning liquor; this concentra-

tion being advantageously as high as 105 220° barkometer. So to speak, the hide is fed with very strong liquor at about the

rate the liquor disappears. The total amount of this liquor employed may be about equal to the white weight of the hides. 110 After the drumming operation is complete the leather may be finished in any of the well known ways.

The present process gives a good yield of 115 good leather in about six days from beam house to bleach. While not in any way restricted to sole leather making, it is particularly advantageous therein. In "acid sole leather" making, it may be applied to the stock from either the first lay-aways or the 120 rockers.

In the accompanying illustration I have shown, more or less diagrammatically, one form of apparatus capable of carrying out the process.

Figure 1 is a central vertical section through a drum;

Fig. 2 is a section along line 2—2 of Fig. 1; and

Fig. 3 is a fragmental section on an en-

70

75

80

85

90

95

100

105

110

120

125

130

larged scale showing the ventilating opening and the splash plate.

In this showing 1 indicates an imperforate drum mounted in bearings 2 and 3 and provided with trunnions 4 and 5. Pulley 6 is keyed to one trunnion. The ends of the drum are provided with openings as at 7 and with dams or splash plates 8 mounted inside the drum by means of bolts 9 and nuts 10 and washers 11. The splash plates are spaced a slight distance from the openings and practically overlap them to some extent. The liquor is introduced into the drum through pipe 12 leading from the source of supply. The interior of the drum is provided with a plurality of pins 13 which serve to catch the hides and assist the tumbling action, the hides being diagrammatically represented in the drum by reference character 14. The operation of this drum is obvious from the foregoing description.

What I claim is:—

1. The process of tanning hides which comprises treating a hide with a small quantity of strong liquor under conditions promoting free evaporation and cooling thereby, and successively supplying fresh small portions of liquor as previous additions tend to disappear by absorption and evaporation until the full quantity of liquor has been supplied and the hide is tanned.

2. The process of tanning hides which comprises agitating the hides in the presence of a small quantity of strong liquor in an apparatus permitting circulation of air therethrough and supplying fresh quantities of liquor as the liquor is absorbed.

3. In the tanning of hides the process which comprises substantially completely absorbing an amount of strong liquor less than that necessary to completely tan the hide and subsequently subjecting the hide to a further quantity of strong liquor, and during the process agitating and cooling the hide.

4. The process of tanning hides which comprises agitating the same in a rotary drum in the presence of an amount of highly concentrated tanning liquor less than that necessary to completely tan the hide, admitting air to the hides during the rotation of the drum to evaporate moisture and cool the hide, and adding further amounts of strong tanning liquor.

5. The process of tanning hides which comprises agitating hides with a small constantly renewed quantity of strong tanning liquor, the amount of such liquor present at any one time being insufficient to prevent free access of air to said hides.

In testimony whereof I affix my signature hereto.

WALTER PETRIE.